

## UNITED STATES PATENT OFFICE.

WILLIAM R. DICKENS, OF COPPERHILL, TENNESSEE.

## LEAD PLATING OF METALS.

No Drawing.

Application filed October 25, 1926. Serial No. 144,190.

This invention relates to the art of lead plating metals, and more particularly ferrous metals, such as iron or steel, and has for its object to provide a method whereby metals may be rapidly, cheaply and effectively lead plated.

I have discovered that metals, and particularly ferrous metals such as iron and steel, after suitable cleaning of impurities and oxides from their surfaces, can be coated with lead by directly welding or burning the lead to the metal with an oxyhydrogen flame, in which flame there is enough hydrogen above what is necessary for combustion to prevent the surface of the metal from becoming oxidized, that is, the oxyhydrogen flame must be one in which the hydrogen exceeds the ratio  $H_2O$ .

In the practice of my invention, I first thoroughly clean the surface by pickling or in any other suitable manner, and with a blow-pipe in one hand and a chemical lead bar in the other I apply the lead to the surface of the metal and simultaneously subject said surface and the lead to the action of an oxyhydrogen flame from the blow-pipe, in which flame the proportion of hydrogen to oxide is in excess of what is necessary to support combustion, that is, is in excess of the ratio  $H_2O$ .

By this action the molten lead is either alloyed to or becomes so closely adherent to the metal that it forms a perfect bond therewith. This results in a preliminary coating and if a thicker coating is desired the same may be added by the ordinary process of welding or "burning" the lead thereon.

I have found that no flux is necessary to obtain a coating of lead on iron or steel, or other metals, but when its use is not prevented by other considerations, an alloy of lead and antimony may be used to obtain a faster welding.

It will be perceived that one of the decided advantages of my process resides in the fact that no special apparatus is required, other than a suitable blow-pipe supplied with oxyhydrogen gas in which the hydro-

gen is in excess of what is necessary to support combustion. 50

What is claimed is:—

1. The method of lead coating metals which consists in simultaneously subjecting the metal surface to be coated and the lead 55 to the action of an oxyhydrogen flame in which the hydrogen exceeds the ratio  $H_2O$ .

2. The method of lead coating metals which consists in applying a bar of chemical lead to the surface to be coated and simultaneously subjecting the lead and metal surface at the point of contact to the action of an oxyhydrogen flame in which the hydrogen exceeds the ratio  $H_2O$ . 60

3. The method of lead coating metals 65 which consists in simultaneously heating the metal surface and flowing molten lead thereover under the action of an oxyhydrogen flame in which the hydrogen exceeds the ratio  $H_2O$ . 70

4. The method of lead coating iron and steel surfaces which consists in cleaning the surface, subjecting the cleaned surface to the action of an oxyhydrogen flame, in which the hydrogen exceeds the ratio  $H_2O$ , and 75 simultaneously melting lead onto said surface by the action of the same flame.

5. The method of lead coating ferrous surfaces which consists in simultaneously heating the ferrous surface and melting the lead 80 while in contact therewith by the action of an oxyhydrogen flame in which the hydrogen exceeds the ratio  $H_2O$ .

6. The method of lead coating ferrous surfaces which consists in simultaneously heating the ferrous surface and melting lead in 85 the presence of antimony while in contact with the ferrous surface by the action of an oxyhydrogen flame in which the hydrogen exceeds the ratio  $H_2O$ . 90

7. The process of coating metal articles with lead which consists in welding the lead to the metal by means of an oxyhydrogen flame in which flame there is present hydrogen in excess of the ratio  $H_2O$ . 95

In testimony whereof I have signed this specification.

WILLIAM R. DICKENS